

Patented Mar. 13, 1928.

1,662,634

# UNITED STATES PATENT OFFICE.

WALTER O. BORCHERDT, OF MOUNTAIN LAKES, NEW JERSEY, ASSIGNOR TO THE NEW JERSEY ZINC COMPANY, OF NEW YORK, N. Y., A CORPORATION OF NEW JERSEY.

## CONCENTRATION OF BARITE.

No Drawing.

Application filed October 19, 1927. Serial No. 227,363.

This invention relates to the concentration of barite from barite ores or other barite-bearing material, and has for its object the provision of an improved process for concentrating barite by selective froth-flotation.

Barite is rather unique among the minerals in that for most of its applications an extremely high degree of purity of the concentrate is required. Lump barite is ordinarily not marketable if it contains less than 38% BaSO<sub>4</sub>, and in some markets a barium sulfate content of less than 92% is not desired. There are both technical and economic reasons for this situation. Some of the common impurities of barite act not only as diluents, causing a degradation of the material, but also have a positive deleterious action because of their influence in the further processes of treatment to which the material is subjected or upon the final product in which the barite is used.

Barite is a relatively soft and friable mineral and in grinding therefore tends to grind finer under given conditions than many of the minerals with which it is associated. Since in ordinary gravity concentration of minerals, sliming is to be specially avoided because of the difficulty of handling the extremely fine-size mineral particles in gravity concentrating machines, this characteristic of the mineral operates commercially to inhibit concentration below a certain range of particle size. It, therefore, has been and is now customary, in the practice of gravity concentration methods, to discard certain products during the concentration of barite ore, despite the fact that they contain a considerable quantity of barite, since the cost of recovering this barite outweighs the possible profit from the operation; in part for the reason before stated, and in part because the impurities with which the barite is associated often have a specific gravity so close to that of the barite itself as to render gravity concentration difficult and uneconomical.

The present invention contemplates the concentration of barite by froth-flotation. In carrying out the invention the barite-bearing material is subjected to froth-flotation in the presence of a barite-selective flotation agent, thereby effecting a substantial concentration of the barite in the result-

ing overflow froth. More particularly, the invention contemplates the provision of a method of concentrating barite by froth-flotation in which high recovery of barite is effected and at the same time a high grade barite concentrate is produced. Thus, the present invention contemplates, with respect to this aspect thereof, an ultimate recovery of at least 60% of the barite in an overflow froth containing not less than 90% barite.

The present invention is based upon my discovery that cotton seed oil pitches are excellent agents for the froth-flotation of barite under proper conditions of application. Cotton seed oil pitches are by-products of the refining of cotton seed oil and they may be obtained commercially in three forms, known respectively as soft, medium and hard pitch. Soft pitch is a liquid; medium pitch is a stiff paste-like substance; and hard pitch is a solid tar-like substance. The soft pitch is slightly miscible in water when heated, and, while it produces some froth when added directly to the flotation cell, it cannot be conveniently used in that manner. The medium and hard pitches are almost entirely immiscible in water, even when heated. I have found that when these substances are used as flotation reagents in solution in gasoline, they give excellent results in barite flotation. The gasoline possesses some frothing power, but by itself does not yield a satisfactory grade of concentrate. The cotton seed oil pitches, when dissolved in gasoline yield copious froths and appear to have a high degree of selective power for barite.

It is well known that certain colloidal constituents of ore pulps are prejudicial or inhibitory to the flotation of sulfids and I have found, likewise, that when barite ores are ground to a size which renders them convenient for treatment by froth-flotation, there generally exists in the pulp colloidal matter which is prejudicial to securing the maximum grade of barite concentrate, the maximum recovery of barite, or both, by froth-flotation.

A large proportion of the barite ore at present mined in the United States is derived from so-called "residual" deposits, and since the gangue in which the barite nodules of such ores occur is principally clay and

earth, it will be understood that barite ores derived from this source contain an unusual amount of colloidal matter.

Barite ores derived from vein or bedded deposits do not generally contain as much colloidal matter as those derived from "residual" deposits, but in the fine grinding of barite ores to the degree required to produce suitable conditions for froth-flotation of the barite, there is almost invariably produced or released a sufficient amount of colloidal material to exercise a deleterious effect upon the froth-flotation treatment of the barite.

In some cases, as where the ore contains a relatively small amount of colloids, it may be sufficient, in order to secure good results, to bring about the deflocculation or dispersion of such colloids preliminarily to flotation, but ordinarily, better results can be secured in all cases by deflocculating and then decanting at least a part of the colloidal constituents associated with the barite ore pulp before the ore is subjected to froth-flotation treatment.

In connection with the preliminary removal of colloids in the concentration of barite ores in order to secure the particularly high grade concentrates which are called for by the barite-consuming trade, the disclosures of my United States Patents No. 1,448,515, dated March 13, 1923, and No. 1,454,838, dated May 8, 1923, are of particular value and importance.

Since barite is a relatively soft and brittle mineral, I find that in barite-bearing log washer tailings, and similar products, and in barite ore pulps which have been ground to a degree suitable to prepare them for flotation, that often considerable of the barite itself becomes colloidal within the meaning which I have assigned to that term in my aforementioned United States patents, to wit, "The colloidal matters may be present as pure colloids, organic or inorganic, or in a state bordering on the so-called 'coarse suspensions.'"

Throughout this specification and the appended claims, I intend to embrace in the expressions "colloids", "colloidal slimes", and "colloidal constituents", both true colloids and those quasi or borderland substances which may not be truly colloidal but partake of the qualities of, or resemble, colloids, and without regard to the sources from which such colloidal matters are derived. Thus, for the purpose of the present invention, the colloidal constituents may be considered as ranging from just above the molecular size upward through the class of so-called suspensoids, which, while possibly not true colloids, still, because of their relatively large specific surface, exhibit some, if not all, of the properties of colloids, and are capable of existing in both the sol or gel state,

or of being dispersed and coagulated or flocculated and deflocculated. By a colloidal slime, therefore, I mean a material which is not necessarily a true colloid, but which exhibits colloidal characteristics to a sufficient degree to make it amenable to the manipulation herein described.

Some of the barite itself generally exists in a colloidal condition in the flotation pulp, and I have found that even when the pulp contains a minimum of other colloidal constituents it is generally desirable to preliminarily remove colloidal constituents, including colloidal barite, before subjecting the barite-bearing ore pulp to froth-flotation treatment, for the reason that colloidal barite floats with extreme ease and it, therefore, tends to unduly armor or coat the bubbles of the froth, producing a condition generally known as "over-stabilization". This condition of over-stabilization, regardless of whether it is brought about by barite or by other colloidal constituents, is an objectionable condition because it tends to mechanically entangle or entrain gangue particles, and to carry them over into the concentrate.

It will be clear from this discussion that in the flotation of barite, colloidal constituents may in several different ways exert a deleterious or undesirable effect. Gangue colloids tend to pass into the froth, thus contaminating the concentrate directly, by reducing its grade, and indirectly by creating over-stabilization of the froth and thus further reducing the concentrate grade by carrying over gangue particles. Such colloids also often exert a direct inhibitory action on the flotation of the coarser particles of barite, causing them to tend to remain in the tailing, thus reducing the recovery of barite. Colloidal barite, while perhaps not in any way interfering with the recovery, does tend, by over-stabilization of the froth, to carry over gangue particles which should remain in the tailing.

The process of deflocculation and decantation, by which the colloidal constituents are in part separated from the ore pulp, depends upon the fact that by dispersing and deflocculating such colloidal constituents they can be held in suspension in quiet pulp. That is, that they can be given a practically zero settling rate, whilst the non-colloidal constituents of the pulp are permitted to settle. In the practice of the process, when sedimentation of the non-colloidal particles has progressed sufficiently, the bulk of the liquid, containing the suspended colloidal constituents and small amounts of extremely fine slow settling non-colloidal constituents, is decanted from the sediment, as described in detail in my United States patents to which reference has been made.

In the case of barite ores, the colloid suspension is often of such character and quan-

5      tity as to justify the recovery of its solids as a by-product. This material contains solids in such an extremely fine state of division that when dried and appropriate-  
 10     ly prepared for the market it is salable as a mineral filler, scouring powder or as "off-color" barites. The colloidal and other solids contained in such a decanted suspension may thus be separated and recovered  
 15     from the water in which they are suspended by flocculating them with appropriate agents and permitting them to settle in the form of a mud or sludge. Or they may be flocculated and separated from the bulk of the water with which they are associated by a froth-flotation treatment, according to the process described in my United States Patent 1,445,989. The solids may be recovered from the aforementioned sludge, or from the colloidal-bearing froth just referred to, by vacuum filtration, or by evaporation of water, or by a combination of these two means.

20      In carrying out my laboratory tests, in cases where no removal of the colloidal constituents of the ore was conducted, I ground a one kilogram (dry weight) sample of the ore in a laboratory ball mill until it was reduced to the desired degree of fineness. I then diluted the sample with water so that the pulp contained about 5½ parts of water to 1 part of ore by weight and placed this pulp in a laboratory flotation machine, or cell, of the pneumatic type.

25      The pulp having been placed in the "rougher" cell, the desired kind and quantity of flotation reagent was added and air was bubbled through the porous blanket, forming with the flotation agent, a barite-bearing froth which was permitted to overflow gently, thus removing the floatable mineral. From time to time samples of the tailing were withdrawn from the cell for examination and returned through the feed pipe, and the liquid coming over with the 30 concentrate froth was separated at intervals and returned to the cell through the feed pipe, thus maintaining a practically constant dilution within the cell and returning part of the flotation agent which was used repeatedly. Further additions of fresh flotation agent were made if and when required and a run was considered complete when the froth no longer contained any considerable quantity of the floatable mineral and when 35 the tailings appeared to be relatively free of such mineral. At this point, the material remaining in the cell was removed and evaporated to dryness, this residue forming the tailing from the test. The concentrate was diluted, as required, and placed in the "cleaner" cell, additional flotation agent being added, if necessary. At the first pass of the "cleaner" a "cleaner" concentrate was made, the material remaining in the cell at 40 the end of the run constituting middling

which was removed and evaporated to dryness. The "cleaner" concentrate was replaced in the "cleaner" cell, diluted with water as required, additional flotation agent added if necessary and again frothed to produce the final or "re-cleaner" concentrate which was evaporated to dryness, whilst the material remaining in the cell, known as the second or "re-cleaner" middling was added to the first or "cleaner" middling and evaporated to dryness. 45

50      When it was desired to deflocculate the colloidal constituents of the ore pulp, I added an appropriate deflocculating agent, generally sodium silicate, either to the pulp before it was ground in the laboratory ball mill or the pulp which was ready for flotation, just enough of the sodium silicate or other deflocculating agent being used to secure the desired result. The deflocculated pulp was then placed in the "rougher" cell and treated as above described.

55      When I desired to remove a portion of the colloid content of the ore, I generally added the required amount of sodium silicate or other deflocculating agent to the ore in the laboratory ball mill, thus grinding the ore in the presence of the deflocculating agent. When the ore was ground to the desired fineness, I diluted with water, forming a pulp in which the colloids were deflocculated. This pulp was allowed to stand quietly in tall cylinders for several hours or until the greater part of the non-colloidal portion of the pulp had settled out. The supernatant 60 colloid-bearing liquor was then carefully decanted. The settled material was re-pulped with an appropriate quantity of water and, if necessary, an additional amount of deflocculating agent was added. These steps were 65 repeated until the colloid content of the pulp had been reduced to the desired extent, which was indicated by experiment, whereupon the final residue was diluted with water and placed in the flotation machine as 70 previously described, while the colloid-bearing liquid, which had been decanted in the several steps above mentioned, was evaporated to dryness. It will thus be seen that starting with a dry weight of one kilogram 75 of feed sample of known composition, I recovered a concentrate, a middling and a tailing product, or a colloid, a concentrate, a middling, and a tailing product from each test. Each of these products was evaporated 80 to dryness, weighed and analyzed, and from the figures so obtained, the grade and recovery were calculated.

85      From many similar tests, the following examples are selected as representatives of the 85 results which may be obtained by practice of the preferred form of the process of the present invention.

90      *Example I.*—Using 25 cc. of a solution of cotton seed oil hard pitch, 10 grams dissolved 90

in 100 cc. of motor gasoline, or at the rate of 5 pounds of hard pitch and 6 gallons of gasoline per ton of material treated, and a feed sample containing 62.5% BaSO<sub>4</sub> and ground to pass 80 mesh, the following results were obtained:

| Sample        | Grams | Per cent of total | Per cent BaSO <sub>4</sub> | Grams BaSO <sub>4</sub> | Per cent of total BaSO <sub>4</sub> |
|---------------|-------|-------------------|----------------------------|-------------------------|-------------------------------------|
| 10            |       |                   |                            |                         |                                     |
| Conc-----     | 500   | 50.0              | 98.28                      | 500                     | 80.5                                |
| Colloids----- | 124   | 12.4              | 61.88                      | 77                      | 12.4                                |
| Mids-----     | 19    | 1.9               | 60.97                      | 12                      | 1.9                                 |
| Tails-----    | 348   | 34.8              | 9.06                       | 32                      | 5.2                                 |
| 15            | 1000  | 100.0             | 62.1                       | 621                     | 100.0                               |

\* Calculated analysis of feed sample.

\* Actual analysis of feed sample.

Example II.—In another test, using 25 cc. of a solution of cotton seed oil hard pitch, 1 gram dissolved in 50 cc. of gasoline, or at the rate of 1 pound of hard pitch and 6 gallons of gasoline per ton of material treated, and a feed sample containing 62.61% BaSO<sub>4</sub> and ground to pass 80 mesh, a barite concentrate containing 97.61% BaSO<sub>4</sub> was obtained with a recovery of 68.60% of the barite contained in the original feed sample.

Example III.—In another test, using 10 cc. of a solution of cotton seed oil medium pitch, 5 grams dissolved in 50 cc. of gasoline, or at the rate of 2 pounds of medium pitch and 2.4 gallons of gasoline per ton of material treated, and a feed sample containing 56.50% BaSO<sub>4</sub> and ground to pass 80 mesh, a barite concentrate containing 96.60% BaSO<sub>4</sub> was obtained with a recovery of 69.20% of the barite contained in the original feed sample.

Example IV.—In another test, using 7 cc. of a solution of cotton seed oil soft pitch, 5 grams dissolved in 50 cc. of gasoline, or at the rate of 1.4 pounds of soft pitch and 1.68 gallons of gasoline per ton of material treated, and a feed sample containing 56.50% BaSO<sub>4</sub> and ground to pass 80 mesh, a barite concentrate containing 97.80% BaSO<sub>4</sub> was obtained with a recovery of 78.10% of the barite contained in the original feed sample.

In its commercial application, the process of the present invention may be carried out in standard froth-flotation machines, either of the so-called agitation type, or of the so-called pneumatic type, or in the machines which represent a combination of the principles of the two preceding types. I prefer to use the pneumatic type machines because of the great capacity which it is possible to secure from a given size machine, and the greater ease of regulation and control. But, as usual in the treatment of minerals by flotation, certain circumstances connected with the ore, the location of the mill, the cost of power and of skilled attendance often indicate some one type of flotation apparatus as

being better suited to the situation than others.

I have found that the degree of comminution to which the barite ore must be subjected to fit it for froth-flotation recovery of its barite content does not differ greatly from that to which sulfid ores intended for flotation are ordinarily reduced. In any event, the ore must be ground fine enough to secure effective severance of the diverse minerals which it contains, and, in general, it is not practicable to float material coarser than that which will pass 35 mesh Tyler standard sieve. Working with a sample of barite-bearing jig tailing from a barite concentrating plant located at Cartersville, Georgia, with which all the conditions of experiment were kept as nearly as practicable indentical, except that the degree of comminution of ore was varied, I found that the degree of comminution in this case, where minerals are practically free from attachment to one another at 35 mesh, had practically no bearing upon the results which could be secured.

I have found that in barite flotation, the considerations respecting dilution of the pulp are the same as they are in the flotation of sulfids. The degree of dilution will depend upon the character of the ore, the fineness of grinding, and similar considerations. Only rarely is the dilution greater than six weights of water per weight of ore, or less than three weights of water per weight of ore. Dense pulp generally gives greater capacity to the flotation machines, but might make it more difficult to secure high grade concentrate and usually a smaller quantity of flotation agent suffices with a dense than with a more dilute pulp.

Barite flotation, according to the process of the present invention, may be carried on in acid, neutral or alkaline pulps, but, because of the wider choice of reagents for deflocculation and flotation which that renders available, it is usually preferable to conduct the flotation in a neutral or alkaline pulp. When, because of other circumstances, such as the natural acidity of the mine water, it is desirable to conduct the flotation on an acid pulp, certain modifications may be necessary if it should be impracticable to neutralize the acidity of the pulp, as by the use of lime.

As is commonly the practice in the flotation of sulfids, it may, in the case of certain barite ores, be necessary to employ certain addition agents for the purpose of properly conditioning the pulp. Thus, it may be necessary to add lime, or some other alkali, to overcome acidity, or sodium silicate, gum arabic, trisodium phosphate, or some similar agent, to secure or maintain deflocculation, as hereinbefore described, the need for such addition agents and their selection necessarily being determined by com-

parative tests, as will be understood by those skilled in the art to which this invention relates.

The temperature of the barite-bearing flotation pulp may, if necessary, be varied as by cooling the pulp by dilution with cold water or by passing it over cooling towers, or by heating it, as by the introduction of steam; but on the score of cost, it is generally desirable to conduct flotation at the natural temperature of the mill water, and, generally, other factors affecting the flotation can be controlled so as to permit of this.

In the practice of the process of the invention, keeping in mind the necessity for producing very high grade concentrate with a maximum recovery at the lowest possible cost for investment and operation, tests should be made on each ore which it is desired to treat, in order to determine the optimum conditions relating to degree of grinding of the ore, deflocculation, or removal of colloids, neutrality, alkalinity or acidity of the pulp, the degree of dilution of the pulp, and its temperature, the agent or agents to be used for conditioning the pulp and securing the barite flotation, and the type of flotation machine.

By means of the process of the present invention, it is possible to produce very high grade barite concentrates with a high percentage recovery of the barite contained in the ore, thus making it possible to improve the grade of barite ores which are now marketable, but whose value can be enhanced by further improving their grade. Ores not heretofore amenable to commercial exploitation can be economically treated for the recovery of their barite content, and waste products of present gravity methods of barite ore dressing can be reclaimed and re-treated.

I claim:

1. The method of concentrating barite-bearing material which comprises subjecting the barite-bearing material in the form of a pulp to a froth flotation operation in the presence of cotton seed oil pitch.

2. The method of concentrating barite-bearing material which comprises adding cotton seed oil pitch dissolved in an appropriate solvent to a pulp of the barite-bearing material, and thereafter subjecting the pulp to a froth flotation operation.

3. The method of concentrating barite-

bearing material which comprises adding cotton seed oil pitch dissolved in gasoline to a pulp of the barite-bearing material, and thereafter subjecting the pulp to a froth flotation operation.

4. The method of concentrating barite-bearing material associated with flocculated colloidal matter in a pulp, which comprises dispersing or deflocculating the colloidal matter, and thereafter subjecting the pulp to a froth flotation operation in the presence of cotton seed oil pitch.

5. The method of concentrating barite-bearing material which comprises grinding the barite-bearing material to flotation size in the presence of sodium silicate, and thereafter subjecting the ground material to a froth flotation operation in the presence of cotton seed oil pitch.

6. The method of concentrating barite-bearing material associated with colloidal matter in a pulp, which comprises removing colloidal matter from the pulp, and thereafter subjecting the pulp to a froth flotation operation in the presence of cotton seed oil pitch.

7. The method of concentrating barite-bearing material associated with flocculated colloidal matter in a pulp, which comprises dispersing or deflocculating the colloidal matter, treating the pulp to remove the dispersed colloidal matter, and thereafter subjecting the pulp to a froth flotation operation in the presence of cotton seed oil pitch.

8. The method of concentrating barite-bearing material associated with flocculated colloidal matter in a pulp, which comprises dispersing or deflocculating the colloidal matter, subjecting the resulting pulp to sedimentation and decantation for the removal of colloidal matter, and thereafter subjecting the pulp to a froth flotation operation in the presence of cotton seed oil pitch.

9. The method of concentrating barite-bearing material which comprises, grinding the barite-bearing material to flotation size in the presence of water and sodium silicate, subjecting the resulting pulp to sedimentation and decantation for the separation and removal of colloidal material, and subjecting the remaining pulp to a froth flotation operation in the presence of cotton seed oil pitch.

In testimony whereof I affix my signature.

WALTER O. BORCHERDT.